# EUROPEAN PATENT SPECIFICATION

(11) **EP 2 503 037 B1**
(45) Date of publication and mention of the grant of the patent: **28.04.2021**
(21) Application number: 11159477.6
(22) Date of filing: 23.03.2011
(51) Int. Cl.: D03D 15/10, D03D 1/02, D03D 15/00, D06M 10/00, D06M 23/08

(54) **A fabric for use in the manufacture of an inflatable air-bag**
Stoff zur Verwendung bei der Herstellung eines aufblasbaren Airbags
Étoffe pour une utilisation dans la fabrication d'un airbag gonflable

(43) Date of publication of application: 26.09.2012
(73) Proprietor: Autoliv Development AB, 447 83 Vårgårda (SE)
(72) Inventor: Kismir, Altay, Windsor, Ontario N8R 2E6 (CA); Stow, David, 41678 Gothenburg (SE); Wootton, Gary, Staffordshire ST7 3PH (GB); Finn, Hugh, Culcheth, WA3 4LG Cheshire (GB); Koehnen, Ralf, Congleton Cheshire CW12 4FJ (GB)
(74) Representative: Forresters IP LLP

(56) References cited:
- EP-A1- 2 500 454
- WO-A1-03/031711
- WO-A1-2004/053213
- JP-A- 62 028 435
- US-A- 3 761 346
- US-A1- 2005 186 873

## Description

THIS INVENTION relates to a fabric for use in the manufacture of an inflatable air-bag, and a method of making the fabric.

Inflatable air-bags, for use in occupant constraint systems in motor vehicles, are conventionally formed from woven fabrics. These fabrics typically comprise two sets of fibres, known as warp and weft fibres, which are interwoven with one another and arranged approximately at right angles to one another. A coating is often applied to such fabrics, and the coating provides the function of decreasing the permeability of the material, and maintaining the fibres in their intended positions.

It is advantageous to reduce the weight of an air-bag as much as possible. This will not only reduce the quantity of material required to construct the air-bag, thereby reducing the cost of the finished item, but will also reduce the weight that must be transported by a vehicle which contains the air-bag.

Focusing on the fabric of an air-bag, there are two principal options for reducing the weight of the air-bag. One is to reduce the weight per unit length of the fibres used to form the fabric (conventionally measured in tex (1 tex = 1 gram per km) or decitex). The other is to reduce the density of fibres per unit area of the fabric (conventionally measured in sett, i.e. threads per cm, counted in as the number of perpendicular threads that are encountered along the length of one of the warp or weft fibres).

If fibres having reduced decitex are used, it is found that the tear and tensile strengths of the fabric are both reduced. This is the case even if the number of threads per unit area is increased to compensate, as each individual thread will break relatively easily.

If the spacing between the fibres is increased, two undesirable effects typically result. The first is that there are larger gaps between the fibres. If the fabric is not coated, then this will increase the permeability of the fabric. If the fabric is covered with a coating, then the coating material will come under greater stress in the larger regions between the fibres when the pressure difference across the fabric is high. Clearly, this leads to an increased risk of rupturing of the coating material.

Secondly, as the sett is reduced, the wrapping angle of each fibre around adjacent fibres is reduced. This reduces the inter-fibre friction, which is fundamental to the formation of the stable fabric. In addition, as stress is applied to the fabric, individual fibres can slide laterally with respect to adjacent fibres, a phenomenon known as combing. For an uncoated fabric, once again this will increase the permeability of the material. For a coated fabric, this combing movement places additional stress on the coating, which will generally lead to micro-ruptures at the elongated interstices.

US2005/186873 discloses compositions and methods for treating textile substrates to obtain superior liquid repellent properties. Durable microscopic surface structures imparted to the fibrous substrate allow liquids to bead up and roll off of its surface. Mechanical abrasion or sanding techniques may be used to create the microscopic surface structures on the surface of a fibrous textile substrate, without substantially breaking fibers, followed by a chemical treatment using, for example, fluorocarbon-containing repellent compositions. Particles may be employed in combination with repellent compositions to achieve superior repellent properties. A property of the roughened surface fibers, the Roughness Factor, is used to characterize the microscopic surface structures on the treated textile surface. Treated textile substrates are disclosed which achieve superior water and oil repellency, even after multiple abrasion or laundering cycles.

US3761346 discloses a composite linear textile material comprises a bundle of filaments having a flexible foam of plastic composition surrounding the bundle, the outer surface of the coating being wrinkled and substantially continuous. The filaments may be continuous glass filaments which may have a protective sizing thereon containing, for example, a wax, a cationic polyester resin, a gelatin and water-repellant substances, or the filaments may be of cotton, polyimides, polyesters, and cellulosics. The coating may be of a vinyl resin such as polyvinyl chloride and the coating composition may contain plasticisers, cell size stabilizers, hand modifiers, fire retardants, pigments and other additives. The fibres may be coated by passing them through a die through which the plastisol formulation is run.

WO2004/053213 discloses a process for forming a continuous filament yarn having the surface tactile character of a spun yarn. The process includes passing the cohesive yarn structure through the interior of a rotating sleeve member disposed in surrounding relation to the cohesive yarn structure. The rotating sleeve member includes an abrasive inner surface of diameter greater than the cohesive yarn structure and is adapted to contact the exterior surface of the cohesive yarn structure such that at least a portion of the elongate filaments disposed at the exterior of the cohesive yarn structure are broken. Terminal ends of the broken filaments define an arrangement of outwardly projecting hairs at discrete locations disposed substantially around the circumference of the cohesive yarn structure. An apparatus for carrying out the process is also provided, as are a continuous filament yarn having characteristics of a spun yarn, and fabrics made from the yarn. WO03/031711 discloses an industrial fabric used in the form of an endless fabric belt to form and convey a nonwoven fiber web during the manufacture of a nonwoven fabric has a web-supporting surface which includes rough-surface yarns which inhibit movement, namely, slippage, of the nonwoven fiber web relative to the web-supporting surface. Preferably, the rough-surface yarns make long floats in one or both directions, that is, lengthwise and/or crosswise, on the web-supporting surface.

JP62028435 discloses an industrial fabric used in the form of an endless fabric belt to form and convey a nonwoven fiber web during the manufacture of a nonwoven fabric has a web-supporting surface which includes rough-surface yarns which inhibit movement, namely, slippage, of the nonwoven fiber web relative to the web-supporting surface. Preferably, the rough-surface yarns make long floats in one or both directions, that is, lengthwise and/or crosswise, on the web-supporting surface.

EP2500454 A1 (state of the art in accordance with Article 54 (3) EPC) discloses a fabric for use in the manufacture of an inflatable air-bag, the fabric comprising interwoven warp fibres and weft fibres which are arranged substantially perpendicular to one another, one or more of the warp and weft fibres being at least partially coated with an adhesive substance to increase the friction between the warp and weft fibres at their intersections The fabric is coated and has a cover factor of 55 % or lower.

EP2500454 A1 further discloses a fabric for use in the manufacture of an inflatable air-bag, the fabric comprising interwoven warp and weft fibres which are arranged substantially at right angles to one another, wherein each of at least one of the warp and weft fibres are formed from a core surrounded by an outer coating.

It is an object of the present invention to provide a fabric for use in the manufacture of an inflatable air-bag which alleviates some or all of the above problems.

Accordingly, one aspect of the present invention provides a fabric for use in the manufacture of an inflatable air-bag, the fabric comprising interwoven warp and weft fibres which are arranged substantially perpendicular to one another, wherein at least one of the warp and weft fibres are formed from two or more filaments which are twisted, wound or assembled together, the fibres having non-uniform cross-sections to increase friction between the fibres at their intersections, the fabric having a cover value below around 55%, and a coating being applied to the fabric to decrease the permeability of the fabric.

Preferably, at least one of the warp and weft fibres are coated with a roughening agent, to increase the surface roughness of the fibres.

A further aspect of the present invention provides an air-bag formed from a fabric according to any preceding claim.

A further aspect of the present invention provides a method of forming a fabric for use in the manufacture of an inflatable air-bag, comprising the steps of: forming at least one set of fibres from two fibre components comprising two or more filaments which are twisted, wound or assembled together; and interweaving the fibres with further fibres to form a fabric having a cover value below around 55%, wherein the fibres and further fibres comprise warp and weft fibres of the fabric and are arranged substantially at right angles to each other; and applying a coating to the fabric to decrease the permeability of the fabric.

Another aspect of the present invention provides a method of manufacturing an air-bag, comprising the steps of: forming a fabric in accordance with the above; and manufacturing the air-bag from the fabric.

In order that the present invention may be more readily understood, embodiments of the invention will now be described, by way of example, with reference to the accompanying drawings, in which:
Figures 1 and 2 show fabrics formed of warp and weft fibres;
Figure 3 shows a treated fibre which may be used in the manufacture of fabrics for use in the construction of an airbag; and
Figure 4 shows a fibre which may be used in the manufacture of fabrics embodying the present invention.

Referring to figure 1, a close-up view of warp and weft fibres 1,2 making up a fabric 3 for use in the manufacture of an inflatable air-bag is shown. Each warp fibre 1 passes alternately under and over weft fibres 2 that are encountered along its length. Similarly, each weft fibre 2 passes alternately under and over warp fibres 1 that are encountered along its length.

The warp and weft fibres 1,2 of the fabric 3 are coated with a substance which increases the friction between the warp and weft fibres 1,2. Preferably, the substance does not produce an adhesive force between the fibres 1,2. In the example shown, the coating comprises solid grains which are adhered to the surfaces of the fibres 1,2, producing an effect which is similar to coating the fibres 1,2 with sand.

If forces are exerted on the warp fibres 1 which would tend to cause the warp fibres 1 to slide with respect to the weft fibres 2, the interaction of the grains will provide a strong resistance to this movement. The result will be an increase in the friction between the warp and weft fibres 1,2 at the junctions 4 therebetween, increasing the overall reliability and stability of the fabric 3.

In further examples, the fibres are treated so that their surfaces acquire a texture, which may be regular or irregular.

One method of achieving this result is to expose the fibres to one or more jets of pressurised air (a technique known as "air texturing"), which imposes dents, ridges and other features in the surfaces of the fibres.

In an alternative technique, the surfaces of the fibres can be treated with a corrosive substance such as an acid, which will remove parts of the outer surface of the fibre, once again leading to surface features and irregularities. In these examples, it may be desirable to use fibres which are heavier than is actually required in the finished article, so that the weight of the fibres is reduced to the required level as part of the fibre surfaces are removed.

If fibres which have been treated in this way are woven to form a fabric as shown in figure 1, the friction between the fibres at their intersections will be significantly increased, as fibres sliding across one another will encounter raised ridges, nodes and projections, which will impede the sliding movement far more than if the fibres simply presented smooth outer surfaces to one another.

In yet further embodiments of the invention, each fibre may be formed from two separate fibre components or filaments. For instance, as shown in figure 4, each fibre 9 may be formed from two or more thinner strands 10, 11, which are wrapped around each other, or interwoven with each other. The strands 10,11 may be formed from the same material, or in alternative embodiments may be formed from different materials.

It will therefore be understood that the term "fibre", when used in this specification, covers individual strands or filaments, as well as arrangements of two or more strands or filaments which are twisted, wound or otherwise assembled together to form a yarn or thread.

It will be understood that forming the fibre 9 from one or more strands 10,11 will increase the surface texture of the fibre 9. If a plurality of such fibres 9 were to be woven into a fabric as shown in figure 1, it will be understood that the fibres 9 would display a high resistance to sliding with respect to one another, as a fibre sliding with respect to a perpendicular fibre will continually encounter ridges which will provide strong resistance to this sliding motion.

It will be understood that all of the above techniques increase the friction between warp and weft fibres where these fibres meet in a woven fabric. This will provide resistance to slippage of the fibres with respect to one another, increasing the stability and reliability of the resulting fabric. If the fabric is uncoated, the permeability of the fabric will remain low when high forces are exerted on the fabric. The fabric is coated, and slippage of the fibres within the coating will be reduced, therefore helping maintain the regular sizes of the interstitial spaces and hence the integrity of the coating under large forces.

The relationship between the amount of material comprising fibres, and the spaces therebetween, per unit area can be calculated, and the result is known as the "cover factor". The cover factor allows fabrics made with different decitex fibres to be compared, and is also a useful way of describing a fabric without specifying a particular decitex value.

In this specification it is stated that fibres are formed or treated to have non-uniform cross-sections. It is appreciated that all fibres, when inspected closely, will have variations in their cross-sections arising from imperfections in the materials from which the fibres are formed, or from the manufacturing process. However, when used in this specification this term refers to deviations from uniformity which are deliberately formed or applied, and are of a magnitude which is over and above those which arise from a standard manufacturing process for fibres of the type which are generally used to weave fabric for vehicle air-bags.

The fabric has a cover value of 55% or lower, and preferably below 54%. These values are lower than those found in conventional air-bag fabrics, but in using techniques described above robust and versatile fabrics having such low cover values are possible.

When used in this specification and claims, the terms "comprises" and "comprising" and variations thereof mean that the specified features, steps or integers are included. The terms are not to be interpreted to exclude the presence of other features, steps or components.

The features disclosed in the foregoing description, or the following claims, or the accompanying drawings, expressed in their specific forms or in terms of a means for performing the disclosed function, or a method or process for attaining the disclosed result, as appropriate, may, separately, or in any combination of such features, be utilised for realising the invention in diverse forms thereof.

## Claims

1. A fabric (3) for use in the manufacture of an inflatable air-bag, the fabric comprising interwoven warp (1) and weft (2) fibres which are arranged substantially perpendicular to one another, wherein at least one of the warp (1) and weft (2) fibres are formed from two or more filaments (10,11) which are twisted, wound or assembled together, the fibres having non-uniform cross-sections to increase friction between the fibres at their intersections, the fabric having a cover value below around 55%, and a coating being applied to the fabric to decrease the permeability of the fabric.

2. A fabric according to claim 1, wherein at least one of the warp (1) and weft (2) fibres are coated with a roughening agent, to increase the surface roughness of the fibres.

3. An air-bag formed from a fabric according to any preceding claim.

4. A method of forming a fabric (3) for use in the manufacture of an inflatable air-bag, comprising the steps of: forming at least one set of fibres from two fibre components comprising two or more filaments (10,11) which are twisted, wound or assembled together; interweaving the fibres (1,2) with further fibres to form a fabric having a cover value below around 55%, wherein the fibres and further fibres comprise warp and weft fibres of the fabric and are arranged substantially at right angles to each other; and applying a coating to the fabric to decrease the permeability of the fabric.

5. A method of manufacturing an air-bag, comprising the steps of: forming a fabric in accordance with claim 4; and manufacturing the air-bag from the fabric.

## Patentansprüche

1. Gewebe (3) zur Verwendung bei der Herstellung eines aufblasbaren Airbags, wobei das Gewebe verflochtene Kett(1)- und Schuss(2)fasern umfasst, die im Wesentlichen senkrecht zueinander angeordnet sind, wobei die Kett(1)- und/oder die Schuss(2)fasern aus zwei oder mehr Filamenten (10,11) ausgebildet sind, die verzwirnt, gedreht oder miteinander zusammengefügt sind, wobei die Fasern uneinheitliche Querschnitte aufweisen, um eine Reibung zwischen den Fasern an ihren Überschneidungen zu erhöhen, wobei das Gewebe einen Bedeckungswert unter etwa 55 % aufweist, und wobei eine Beschichtung auf das Gewebe aufgebracht wird, um die Durchlässigkeit des Gewebes zu verringern.

2. Gewebe nach Anspruch 1, wobei die Kett(1)- und/oder die Schuss(2)fasern mit einem Aufraumittel beschichtet sind, um die Oberflächenrauheit der Fasern zu erhöhen.

3. Airbag, der aus einem Gewebe nach einem der vorhergehenden Ansprüche ausgebildet ist.

4. Verfahren zum Ausbilden eines Gewebes (3) zur Verwendung bei der Herstellung eines aufblasbaren Airbags, das die folgenden Schritte umfasst:
Ausbilden wenigstens eines Satzes von Fasern aus zwei Faserkomponenten, die zwei oder mehr Filamente (10,11) umfassen, die verzwirnt, gedreht oder miteinander zusammengefügt sind;
Verweben der Fasern (1,2) mit weiteren Fasern, um ein Gewebe auszubilden, das einen Bedeckungswert unter etwa 55 % aufweist, wobei die Fasern und die weiteren Fasern Kett- und Schussfasern des Gewebes umfassen und im Wesentlichen in rechten Winkeln zueinander angeordnet sind; und
Aufbringen einer Beschichtung auf das Gewebe, um die Durchlässigkeit des Gewebes zu verringern.

5. Verfahren zum Herstellen eines Airbags, das die folgenden Schritte umfasst:
Ausbilden eines Gewebes nach Anspruch 4; und
Herstellen des Airbags aus dem Gewebe.

## Revendications

1. Tissu (3) destiné à être utilisé dans la fabrication d'un coussin de sécurité gonflable pneumatique, le tissu comprenant des fibres de chaîne (1) et de trame (2) entrelacées qui sont disposées sensiblement perpendiculairement les unes aux autres, les fibres de chaîne (1) et/ou de trame (2) étant formées de deux ou plusieurs filaments (10, 11) qui sont torsadés, enroulés ou assemblés ensemble, les fibres ayant des sections transversales non uniformes pour augmenter le frottement entre les fibres à leurs intersections, le tissu ayant une valeur de couverture inférieure à environ 55 %, et un revêtement étant appliqué sur le tissu pour diminuer la perméabilité du tissu.

2. Tissu selon la revendication 1, dans lequel les fibres de chaîne (1) et/ou de trame (2) sont revêtues d'un agent de rugosité, pour augmenter la rugosité de surface des fibres.

3. Coussin de sécurité gonflable formé à partir d'un tissu selon l'une quelconque des revendications précédentes.

4. Procédé de formation d'un tissu (3) destiné à être utilisé dans la fabrication d'un coussin de sécurité gonflable pneumatique, comprenant les étapes consistant à :
former au moins un ensemble de fibres à partir de deux éléments de fibres comprenant deux ou plusieurs filaments (10, 11) qui sont torsadés, enroulés ou assemblés ensemble ;
entrelacer les fibres (1, 2) avec d'autres fibres pour former un tissu ayant une valeur de couverture inférieure à environ 55 %, les fibres et des fibres supplémentaires comprenant des fibres de chaîne et de trame du tissu et étant disposées sensiblement à angles droits les unes par rapport aux autres ; et
appliquer un revêtement sur le tissu pour diminuer la perméabilité du tissu.

5. Procédé de fabrication d'un coussin de sécurité gonflable, comprenant les étapes consistant à :
former un tissu selon la revendication 4 ; et
fabriquer le coussin de sécurité gonflable à partir du tissu.
